

Patented May 19, 1925.

1,538,431

# UNITED STATES PATENT OFFICE.

SIGURD GIERTSEN, OF CHRISTIANSSANDS, NORWAY, ASSIGNOR TO KRISTIANSSANDS NIKKELRAFFINEBINGSVERKE, OF CHRISTIANSSANDS-S., NORWAY, A CORPORATION OF NORWAY.

## COPPER-NICKEL ANODE AND METHOD OF PREPARING THE SAME.

No Drawing.

Application filed September 26, 1921. Serial No. 508,359.

To all whom it may concern:

Be it known that I, SIGURD GIERTSEN, a citizen of Norway, residing at Christiansands-S., Norway, have invented certain new and useful Improvements in Copper-Nickel Anodes and Methods of Preparing the Same; and I do hereby declare the following to be a full, clear, and exact description of the invention, such as will enable others skilled in the art to which it appertains to make and use the same.

This invention relates to improvements in copper-nickel anodes, etc., as well as in the method of their production, and in the refining of Bessemerized copper-nickel matte, etc.

In making copper-nickel anodes for electrolytic refining from Bessemerized copper-nickel matte, the present method consists in pulverizing the matte, roasting the pulverized matte for the removal of sulfur, thereby converting the metals into the form of oxides, and smelting the resulting oxides to produce metal containing only a small percentage of sulfur, and finally casting such metal into anodes.

I have now found that the production of copper-nickel anodes from Bessemerized copper-nickel matte can be greatly simplified, and that an anode having characteristic composition and properties, and well adapted for use in electrolytic refining, can be readily produced without the roasting and subsequent smelting operations now used.

I have found that, by continuing the blowing operation in the Bessemer converter after the iron is slagged off, a sufficient amount of sulfur can be removed so that the resulting metal composition can be cast into anodes directly from the converter, and the anodes will be of sufficient toughness for use in electrolytic refining, and can be made of appropriate composition for such use. Ordinarily, prolonged blowing in the converter results in freezing the charge, but I have found that by adding to the charge a small amount of scrap iron or other heat-producing material, such as ferro-silicon, sufficient additional heat will be supplied by oxidation to permit the sulfur to be gradually lowered to a degree considerably below that otherwise commercially feasible. A small quantity of low-grade matte or pyrrhotite ore is particularly well adapted for use as heat producing material, since such materials

seem to give off their sulfur very quickly, leaving the iron to oxidize and thereby supply the supplemental heat. By thus prolonging the blowing operation, it is possible to produce a metal of sufficient toughness for anode making, and containing less than 10% of sulfur, e. g. about 8 to 10% or less.

The metal thus produced can be directly cast into anodes from the converter. The anodes thus produced are well adapted for use in the electrolytic production of nickel.

Instead of casting the metal into anodes, it can be otherwise used in the refining of copper-nickel matte. The metal may thus be pulverized and used for cementing out copper from copper-nickel sulfate solutions, or as raw material for further refining by other processes.

I claim.

1. The improvement in the Bessemerizing of copper-nickel matte, which comprises continuing the blowing of the charge after practically all iron has been removed and maintaining the charge at a sufficient temperature by the addition of heat producing material.

2. The improvement in the Bessemerizing of copper-nickel matte, which comprises continuing the blowing of the charge after practically all iron has been removed and maintaining the charge at a sufficient temperature by the addition of iron or material containing iron which is oxidized and slagged off.

3. The method of producing copper-nickel anodes, which comprises subjecting copper-nickel matte to a Bessemerizing operation, continuing the blowing of the charge after practically all iron has been removed while maintaining the charge at a sufficient temperature by the addition of a heat producing material, until the metal has a composition adapted for making into anodes, and casting the resulting metal into anodes.

4. The method of producing copper-nickel anodes, which comprises subjecting copper-nickel matte to a Bessemerizing operation, continuing the blowing of the charge after practically all iron has been removed, while maintaining the charge at a sufficient temperature by the addition of a heat producing material, until the sulfur content has been reduced to below 10% and casting the resulting metal into anodes.

5. The improvement in the electrolytic

refining of nickel, which comprises carrying out the electrolytic operation with a copper-nickel anode of metal produced in the Bessemer converter by adding a heat producing material and prolonging the blowing and containing less than about 10% of sulfur.

6. The improvement in the purifying of copper nickel sulfate solutions by cementation which comprises subjecting such solution to the action of metal produced in the Bessemer converter after the addition of a

heat producing material and containing less than about 10% of sulfur.

7. The improvement in the Bessemerizing of copper-nickel matte, which comprises continuing the blowing of the charge after practically all iron has been removed and maintaining the charge at a sufficient temperature by the addition of ferrosilicon.

In testimony whereof I affix my signature.

SIGURD GIERTSEN.